

Jan. 11, 1938.

H. MUELLER ET AL

2,104,906

MEANS FOR CASTING ROLLS

Filed April 6, 1935

2 Sheets-Sheet 1

FIG. 1.



FIG. 2.



WITNESSES  
A. B. Wallace.  
E. O. Johns

BY

INVENTORS  
Henry Mueller  
Harry E. Walters  
Brown, Gitchell & Rieck

ATTORNEYS.

Jan. 11, 1938.

H. MUELLER ET AL  
MEANS FOR CASTING ROLLS

2,104,906

Filed April 6, 1935

2 Sheets-Sheet 2

FIG. 3.



WITNESSES  
A. B. Wallace  
E. O. Johns

BY

INVENTORS  
Henry Mueller  
Harry E. Walters  
Brown, Critchlow & Flick  
ATTORNEY.

## UNITED STATES PATENT OFFICE

2,104,906

## MEANS FOR CASTING ROLLS

Henry Mueller and Harry E. Walters, Pittsburgh,  
Pa., assignors to United Engineering & Foundry  
Company, Pittsburgh, Pa., a corporation of  
Pennsylvania

Application April 6, 1935, Serial No. 15,028

5 Claims. (Cl. 22—127)

This invention relates to the manufacture of castings from metal which shrinks upon solidifying, and is more particularly concerned with apparatus for casting rolls for use in rolling mills.

5 In the casting of rolling mill rolls and the like, it is necessary to produce rolls free from blow-holes, piping, segregations, pockets and other casting faults. Likewise it is of paramount importance to reduce the machining requisite after 10 casting to a minimum to save material and labor costs.

15 However, in vertically casting, substantially to form and size, a roll having a heavy central body portion and reduced bearing necks on either end, the metal in the neck portions solidifies before the metal in the heavy middle portion of the roll. This results in the formation of a pocket or fissure just where the upper neck portion joins the middle portion of the roll. Thus the 20 strength of the casting is greatly reduced just at the point where the most strength is needed, and as a result roll failure has often occurred at these points of weakness which has led to the scrapping of poorly cast rolls.

25 It has been proposed to eliminate the pocket or fissure by casting the roll with bearing necks of considerably greater diameter than the diameter of the bearing neck after machining and as used on the roll. In this practice the bearing neck may even be cast the same diameter as the body portion of the roll. Methods of this character may improve the strength and solidness of the casting, but much more metal is required and subsequent removal of this excess material, to 35 bring the bearing necks to size, necessitates lengthy and expensive machining operations so that roll cost is high.

30 Extra long or high risers have also been suggested but their use entails extra material in the casting which must be sheared or machined off and scrapped and moreover difficulty in the formation of pockets and fissures is still encountered.

40 It is the object of our invention to avoid and overcome the foregoing and other difficulties of prior practices and to provide improved commercially feasible apparatus for casting rolls free of casting faults and requiring little machining.

45 Our invention is predicated on our discovery that a roll with reduced bearing necks can be cast substantially to form in a sand mold without the formation of casting faults so long as the heat is bled or removed in a controlled manner from the lower bearing neck and large central portion of the roll while insuring that the 50 heat will be retained in the upper bearing neck

to keep it liquid until the lower bearing neck and the central portion of the casting freeze.

In the practice of our invention we provide a 5 molding flask having substantially only heat insulating material defining a molding cavity positioned so the axis of the cast roll is substantially vertical. The heat insulating means adjacent the upper neck portion of the casting has a relatively high resistance to the passage 10 of heat and is substantially thick so that it functions to maintain the upper roll neck molten for a considerable period after casting. The heat insulating means adjacent the remaining portions of the casting have a medium resistance to the passage of heat and are relatively thin and 15 have high heat conductive means positioned directly behind them to absorb and conduct away, in a rapid manner but without chilling, the heat of the lower bearing neck and the enlarged central portion of the roll casting. Thus these 20 portions will freeze in the order named and before the upper bearing neck to produce a sound casting and one which will necessitate little machining and scrap, and which will have a very solid 25 and sound connection between the upper bearing neck and the central portion of the roll.

25 Apparatus which may be and has been used in the practice of our invention as just explained is illustrated in the accompanying drawings, of 30 which Fig. 1 is a vertical cross-sectional view of a molding flask and casting constructed in accordance with the principles of the invention; Fig. 2 is a fragmentary cross-sectional view of a portion of Fig. 1, but illustrating a modification 35 of the construction thereof; and Fig. 3 is a vertical cross-sectional view similar to Fig. 1, but illustrating another embodiment of the invention.

35 Referring to the particular embodiment of our invention seen in Fig. 1 of the drawings, the numeral 10 indicates generally a flask, which may 40 be of any standard type, but which preferably comprises a plurality of endless ring portions 12, 14, 16 and 18 secured one on top of another in any suitable way as by the usual flask clamps (not shown).

45 The flask 10 carries molding sand 20, or other similar material, which defines the contour of the mold and shapes the roll, indicated generally at 28. The mill roll 28 comprises an enlarged central portion 30 with reduced neck bearing portions 32 and 34. The neck portion 34 is extended 50 vertically to provide a riser or head 36 in accordance with the usual practice. The dotted lines 40 indicate the contour to which the casting 28 is preferably machined.

It will be seen from the drawings that the ring 16 of the flask 10 is made in the form of a heavy chill which has substantially the same volume of metal as the heavy central portion 30 of the roll casting 28. This heavy chill ring 16 does not function in the nature of a true chill, to form the casting 28 with a hardened surface, as the chilling action is definitely prevented by the layer of sand 20a coating the surface of the chill ring 16. By 10 avoiding the true chilling action and having instead a heat bleeding operation as hereafter explained, we prevent the formation of surface cracks on the cast roll which are very undesirable because of necessity for heavy machining and 15 danger of roll failure from the cracks and at the same time provide means whereby the amount of heat removed from the casting can be predetermined and controlled.

The resistance of the layer of sand 20a to the 20 passage of heat is very carefully determined, either by actual experiment, by calculation, or by both, to reach a conclusion as to its proper thickness. In all events the thickness is such that the heat from the thickened portion 30 of the roll casting 28 will be drawn to the chill ring 16 in an even steady flow which will cause the solidification of the central enlarged portion 30 shortly after the solidification of the lower bearing neck 32.

30 We have found that when casting a roll having a centrally enlarged portion from about two to about five feet in diameter the sand layer 20a should be about three-quarters of an inch thick for the smaller size rolls and should increase in thickness proportionally for the larger size rolls with the sand being about one and one-half inches thick for the largest rolls. The sand, or other molding material, forming the layer 20a should have a thermal conductivity of approximately 35 three B. t. u. when used in the thicknesses described just above. (Thermal conductivity is the number of British thermal units passing through a one-inch thick layer of the material one foot square with a one degree Fahrenheit temperature difference on opposite sides of the layer.) This compares with a thermal conductivity of over 40 three hundred B. t. u. for steel.

The lower bearing neck 32 of the casting 28 is adapted to be solidified first in the freezing of the 50 casting, and this is accomplished in the embodiment of the invention illustrated by the provision of chill rings 44 and 46 adjacent to the portion 32. As will be seen from the drawings the chill rings 44 and 46 are not placed directly in contact with 55 the surface of the casting which would chill and harden the casting surface, but they are spaced from the casting by a covering layer 20b of molding sand. This molding sand layer 20b functions similarly to the layer 20a above described in that 60 it serves as a refractory or insulating layer between the chills and the casting, and permits a gradual withdrawal of the heat from the neck portion 32 without chilling the surface of the neck portion. The character and thickness of the 65 layer 20b can be determined by the same standards as the layer 20a.

It is important that the thickness of the sand 70 layer 20b be carefully determined either analytically, experimentally, or both, so that the heat bleeding chills will draw off the desired amount of heat from the neck portion in the desired time interval. Likewise, the diameter of the chill rings 44 and 46 is preferably such that they substantially equal the volume of the associated neck 75

portions. We have found that chill rings of approximately the character described give the best results. However, it is possible to increase the size of the chills 44 and 46 and even to make them part of ring 18 so long as the bleeding of heat 5 from the lower bearing 32 follows the teachings of our invention. The chill or heat withdrawing rings 16, 44 and 46 are preferably of cast iron or other material having a thermal conductivity of at least two hundred B. t. u. 10

The upper neck portion 34 of the casting 28 is adapted to be kept in a molten condition until after the solidification in turn of the bearing neck 32 and the main central portion 30 of the casting 28. This is achieved by providing 15 a relatively thick refractory layer 50 at the upper end of the mold, which refractory may comprise any suitable heat insulating material having a thermal conductivity of not over approximately two and preferably about three-quarters B. t. u. 20 By way of example, we employ a calcined semi-refractory type of diatomaceous silica. This material as mined is substantially of the composition which we employ. However, to assist in the molding thereof, we preferably grind the material 25 and mix it with fire clay which functions as a binder.

In using the apparatus just described in the manufacture of a mill roll, the mold is first made up in the usual manner with the axis of the mold 30 substantially vertical. The steel is then cast in the mold, by any well-known way, as for example, by bottom pouring with the aid of tangentially extending gates (not shown) connected to the bottom of the molding cavity. When the cast- 35 ing is completely poured, the heat withdrawing or chill rings 44 and 46 first cause the neck portion 32 of the casting to freeze with freezing extending gradually upwardly as occasioned by the heat withdrawing or chill ring 16. The refractory 40 and heat insulating layer 50 prevent the premature freezing of the neck portion 34 as the casting solidifies from the bottom upwardly, and impurities, inclusions and the like are carried to the very top of the riser or head 36 with the formation of only a relatively short pipe. The formation of a fissure or pocket at the junction of the upper bearing neck and the central portion of the roll is completely avoided. 45

In the modification of the invention illustrated 50 in Fig. 2, the thickness of the sand layer 20a of Fig. 1 has been changed so that the layer, indicated by the numeral 201a in Fig. 2, gradually increases in thickness upwardly of the mold. This still further insures freezing of the casting 55 from the bottom gradually up to the top in that the most heat will be withdrawn from the casting at and near its bottom with the heat bleeding control layer of sand 201a getting thicker upwardly of the casting and finally becoming a distinct insulating layer and merging into the heat insulating refractory 501 at the juncture of the upper bearing neck and the roll body. The chill ring 161 associated with the tapered-thickness sand layer 201a is appropriately tapered also. 60 The chill ring adjacent the lower bearing neck is numbered 441, and the flask and sand are identified as 141, 181 and 201, respectively. 65

Now referring to the embodiment of the invention illustrated in Fig. 3, the numeral 60 indicates generally a vertically positioned cylindrical flask filled with molding sand 62 which carries and supports cooling rings 64, 66 and 68. These cooling rings are preferably made of welded steel, 75

and are, in the embodiment shown, in the form of hollow cylinders. Conduit means 70 are connected to the bottom of the cooling ring 64 and function to supply a cooling fluid such as water thereto. Conduits 72 and 74 connect the various cooling rings together while a conduit 76 functions to carry the cooling fluid from the rings. Vanes 78 are preferably formed in conjunction with the cooling rings to prevent the collapse of the walls thereof and to assist in distributing the water or other cooling fluid around the cooling rings. The thermal conductivity of the cooling rings will be quite high and obviously well in excess of two hundred B. t. u. dependent upon 10 the flow of cooling fluid therethrough.

Positioned at the top of the cooling rings is a cylindrical, relatively thick layer 80 of heat insulating material which is held in the flask with the aid of the surrounding molding sand 62, or if 20 desired, gagers 82, or other similar means, can be secured in the insulating body 80 to extend into the molding sand to assist in holding the insulating body in the mold. The composition, 25 dimensions, and function of the insulating layer 80 are similar to those above described in conjunction with the heat insulating layer 50 shown in Fig. 1.

The numeral 86 indicates generally a steel casting having an enlarged central portion 88, a reduced lower bearing neck 89 and a reduced upper bearing neck 90 which extends into a riser or head 92 of the casting. The dotted lines 94 indicate generally the contour of the machined roll obtained from the casting 86.

35 Positioned between the cooling rings 64, 66 and 68 and the casting 86 are layers 62a and 62b of molding sand which prevent direct contact and chilling of the metal of the casting against the cooling rings. The thickness of the sand layers 40 62a and 62b is such that they permit the controlled withdrawing of heat from the casting portions. The composition, thickness and function of the layers 62a and 62b are similar to those described above for layers 20a and 20b.

45 The casting may be poured in any suitable manner, but preferably is bottom poured with the aid of one or more gates 96 positioned tangentially of the molding surface of the neck portion 89. The size of the flask 60 can be increased 50 at one corner, for example, to permit the inclusion of a vertical passage from the gates 96 to the top of the flask. This has not been illustrated in the drawings as bottom pouring is old and well known.

55 The modification of the invention shown in Fig. 2 and relating to the tapered thickness of the sand or insulating layer between the casting and the heat withdrawing means may be applied also to the apparatus of Fig. 3 as will be understood.

In practicing our invention with the apparatus just described, the mold is made up in the standard manner and in the form set forth, and the casting is poured in accordance with the usual 65 procedure. We then begin to pass cooling fluid to and through the cooling chambers 64, 66 and 68 after the casting has been completely poured. Therefore any possible danger is prevented which might result if the water were in the cooling 70 rings during the pouring with the water leaking through into contact with the molten metal. It will be appreciated that the cooling rings are very carefully manufactured and tested under high pressures so that chances for escape of

water and contact with the molten metal can safely be said to be eliminated.

As indicated in the drawings by the arrows, cooling fluid passing through the rings 64, 66, and 68 is introduced into the bottom ring 64 by 5 means of conduit 70, passes through the lower rings, on up through the remaining rings in turn and finally discharges through conduit 76. This insures that the most cooling action is achieved at the lower end of the casting with the cooling 10 fluid gradually warming as it is carried upwardly through the cooling rings. Thus freezing of the cast roll will gradually take place from the bottom upwardly.

The heat insulating body 80 prevents the escape 15 of heat from the upper neck portion 90 and the riser 92 and together with the cooling rings insures that the upper neck portion is the last to freeze in the casting. In this manner all slag, blow-holes and the like are carried upwardly 20 and finally form a small pipe at the top of the riser as is illustrated. The casting, and particularly the joinder of the upper bearing neck and the central portion of the roll, is very solid and 25 free of air pockets, impurities, segregations, blow-holes and the like and when machined down to the dotted lines 94 provides a very high-grade mill roll.

From the foregoing description it will be apparent that improved apparatus for casting 30 metals, such as steel, which shrink on cooling, has been provided, and that more particularly improved apparatus for the manufacture of mill rolls is provided. The disadvantages and undesirable features of prior known practices have 35 been avoided. Moreover, the apparatus is relatively inexpensive and requires no complicated heating structures and is readily incorporated in standard molding flasks.

While we have illustrated only certain particular embodiments of the invention, it will be appreciated that the invention is not limited thereto or thereby but is defined in the appended claims.

We claim:

1. Apparatus for casting mill rolls or the like, including a flask, heat insulating means completely defining a molding cavity in the flask, the cavity being positioned so the axis of the cast roll is substantially vertical, said heat insulating means surrounding the upper neck portion of the casting being substantially thick and adapted to maintain the surrounded portion of the casting molten, the heat insulating means adjacent substantially all the remaining portions of the casting 50 being less resistant to the passage of heat, and also relatively thin, and high heat conductive means positioned directly behind the last referred to heat insulating means for readily absorbing and conducting away heat passing there- 55 through.

2. Apparatus for casting mill rolls or the like including heat insulating means defining a molding cavity positioned so the axis of the cast roll is substantially vertical, the heat insulating 65 means adjacent the upper neck portion of the casting being substantially thick and adapted to maintain the surrounded portion of the casting molten, the heat insulating means adjacent the remaining portions of the casting being less resis- 70 tant to the passage of heat and also relatively thin, and high heat conductive means positioned directly behind the last referred to heat insulating means for readily absorbing and conducting away heat passing therethrough, said heat con- 75

ductive means including metal jackets with cooling fluid circulated therethrough.

3. Apparatus for casting mill rolls or the like including a flask, heat insulating means defining a molding cavity positioned so the axis of the cast roll is substantially vertical, said heat insulating means surrounding the upper neck portion of the casting having a thermal conductivity of approximately three-quarters B. t. u. and being substantially thick and adapted to maintain the surrounded portion of the casting molten, the heat insulating means adjacent the remaining portions of the casting having a thermal conductivity of approximately three B. t. u. and being relatively thin, and high heat conductive means, having a thermal conductivity of at least approximately two hundred B. t. u., positioned directly behind the last referred to heating insulating means for readily absorbing and conducting away heat passing therethrough, said heat conductive means including metal bodies substantially equal in volume to the opposed volume of the casting.

4. Apparatus for casting mill rolls or the like including a flask, heat insulating means defining a molding cavity positioned so the axis

of the cast roll is substantially vertical, said heat insulating means adjacent the upper neck portion of the casting having a thermal conductivity of approximately three-quarters B. t. u. and being substantially thick and adapted to maintain the surrounded portion of the casting molten, the heat insulating means adjacent the remaining portions of the casting having a thermal conductivity of approximately three B. t. u., and being between three-quarters and one and one-half inches thick, and high heat conductive means, having a thermal conductivity of at least approximately two hundred B. t. u., positioned directly behind the last referred to heat insulating means for readily absorbing and conducting away heat passing therethrough.

5. In a mold for casting mill rolls and like articles in a vertical position, heat removing means adjacent the casting for cooling the casting, and insulating means of increasing thickness upwardly of the casting positioned between the heat removing means and the casting for reducing and controlling the flow of heat to the removing means.

HENRY MUELLER. 25  
HARRY E. WALTERS.